

# United States Patent [19]

Jorek et al.

[11] 3,914,496

[45] Oct. 21, 1975

[54] ANTISTATIC FINISHING OF SURFACES

[75] Inventors: **Helmut Jorek; Rolf Fikentscher**,  
both of Ludwigshafen; **Joachim  
Kurze**, Leutershausen, all of  
Germany; **Herbert Helfert**, Trenton,  
Mich.  
[73] Assignee: **Basf Aktiengesellschaft**,  
Ludwigshafen (Rhine), Germany

[22] Filed: **Mar. 1, 1974**

[21] Appl. No.: **447,228**

[30] Foreign Application Priority Data

Mar. 1, 1973 Germany ..... 2310186

[52] U.S. Cl. ..... **428/279; 252/8.6; 252/8.7;  
260/459 R; 260/459 A; 260/501.15;  
260/567.6 R; 260/567.6 M**

[51] Int. Cl.<sup>2</sup> ..... **C08J 1/44**

[58] Field of Search ..... 117/139.5 CQ, 138.8 N,  
117/138.8 UA, 138.8 B; 252/8.6, 8.7;  
260/567.6 R, 567.6 M, 459 R, 459 A,  
501.15; 428/279

[56]

References Cited

UNITED STATES PATENTS

|           |         |                   |              |
|-----------|---------|-------------------|--------------|
| 2,096,749 | 10/1937 | Kritchevsky.....  | 117/139.5 F  |
| 2,205,042 | 6/1940  | Lenher et al..... | 117/139.5 F  |
| 3,065,110 | 11/1962 | Hagge et al. .... | 117/138.8 UA |
| 3,174,985 | 3/1965  | Berger .....      | 117/138.8 N  |
| 3,684,567 | 8/1972  | Roth.....         | 117/139.5 CQ |

Primary Examiner—Michael R. Lusignan  
Attorney, Agent, or Firm—Johnston, Keil, Thompson  
and Shurtleff

[57]

ABSTRACT

Antistatic finishing of surfaces of shaped articles, especially textiles, which tend to acquire an electrostatic charge, using quaternary ammonium compounds which contain 2 to 4 hydroxyethyl groups per ammonium group.

2 Claims, No Drawings

## ANTISTATIC FINISHING OF SURFACES

This invention relates to the antistatic finishing of surfaces of shaped articles, especially textiles, which tend to acquire an electrostatic charge, using quaternary ammonium compounds which contain 2 to 4 hydroxyethyl groups per ammonium group.

It is known that many articles consisting of macromolecular materials tend to build up an objectionable electrostatic charge during processing or in use. This tendency is particularly common with articles of synthetic macromolecular materials; however, it is not restricted to these but also occurs with fibers of cellulose esters and even fibers of cellulose, regenerated cellulose, silk, wool and other vegetable and animal products, when the moisture content of these fibers - which is primarily determined by the relative atmospheric humidity - falls below a certain limit. This limit differs from one type of fiber to another.

Numerous chemical compounds have already been proposed as antistatic agents. The conventional antistatic agents are mostly longchain alkyl or aralkyl compounds of the non-ionic, anionic or cationic type. Amongst these, the cationic fatty alkyl compounds of nitrogen or phosphorus, in the form of their tertiary or quaternary salts, are preferred because — by virtue of their substantivity and their orientability on the surface of the fiber — they produce very good antistatic effects. The orientation of the molecules of these surface-active positively charged compounds is attributable to their chemical structure which is characterized by a long hydrophobic alkyl radical of 8 to 20 carbon atoms and a hydrophilic salt-forming group. A cycloaliphatic or aromatic radical can take the place of the longchain alkyl radical, but, evidently for steric reasons, these products are less effective antistatic agents than the aliphatic compounds.

The disadvantage of these compounds is that they are strongly cationic, hence react both with anionic surfactants and with anionic dyes to form sparingly soluble salts, and therefore cannot be used conjointly with such surfactants or dyes.

Compounds which act as antistatic agents and, in spite of their pronounced positive charge, do not react as cationic compounds have been disclosed in the literature. These are substituted urea derivatives which, however, suffer from the disadvantage — when used on textiles — that the substrate finished with them can develop an unpleasant fishy odor on storage under adverse conditions.

It is an object of the present invention to provide a process for antistatic finishing, especially of textiles, which is at least as good as the conventional processes in respect of antistatic activity but does not suffer from the disadvantages described.

We have found a process for antistatic finishing of surfaces of shaped articles which tend to build up an electrostatic charge, by coating with ammonium salts, wherein the coating agents used are ammonium salts of the formula



where  $X^-$  is a monovalent organic or inorganic anion or the  $n$ -th part of an  $n$ -valent anion of a water-soluble

acid, (i.e., one equivalent of an anion of a water-soluble acid) R and Q independently of one another are each hydroxyalkyl of 2 or 3 carbon atoms, alkyl of 1 to 6 carbon atoms or benzyl and Q can also be the radical



in which A is alkylene of 2 to 6 carbon atoms. Compounds of the said formula in which R is hydroxyethyl and Q is methyl or ethyl are preferred.

The compounds can be obtained conventionally by reaction of appropriately substituted diethanolamines or of triethanolamine with alkylating, hydroxyalkylating or benzylating agents, such as dialkyl sulfates, alkyl halides or alkyl dihalides, toluenesulfonic acid alkyl esters, benzyl chloride or ethylene oxide or propylene oxide together with acids, in equimolar ratios. The quaternization reactions take place at temperatures of 20° to 100°C though with some sluggish quaternizing agents temperatures of up to 150°C are required. Solvents can be used — for example for the purpose of cooling the mixture through boiling of the solvent.

As the anion  $X^-$  it is possible to use more or less any watersoluble organic or inorganic acid radicals. For economic reasons, the anions of industrially available acids, for example of sulfuric acid, hydrochloric acid, hydrobromic acid, toluenesulfonic acid and methylsulfuric acid are preferred.

Compounds with fewer than two 2-hydroxyethyl groups on the quaternary nitrogen are not sufficiently active antistatically.

The compounds, and their manufacture, are not claimed herein.

In contrast to the quaternary ammonium compounds conventionally used for this purpose, the compounds of the formula shown exhibit an antistatic action, even at low relative atmospheric humidities, to a hitherto unknown degree. They are therefore particularly suitable for the antistatic finishing of fibrous textile materials of all kinds, for example fibers, filaments, tops, card slivers, yarns, non-woven fabrics, felts, woven fabrics and knitted fabrics, consisting of synthetic high molecular materials, such as linear polyesters, polyamides, acrylonitrile polymers, polyolefins and polyvinyl compounds, or consisting of natural high molecular weight materials or their derivatives, such as cellulose, regenerated cellulose, cellulose esters, silk, wool and other vegetable and animal materials.

The antistatic effect of the compounds persists for a prolonged period even at high temperatures; textile materials finished with these compounds do not yellow, because of the high heat stability of the compounds. In spite of their pronounced positive charge the compounds do not behave as cationic compounds, that is to say they react neither with anionic surfactant nor with anionic dyes to form precipitates, so that they are universally applicable without the hazard of the difficulties which arise, when using the conventional cationic antistatic compounds, during subsequent finishing processes such as dyeing, wash-and wear finishing and hydrophobic treatments. Their particular advantage is that even on storing the finished textiles under adverse conditions a fishy odor does not develop.

In addition, these antistatic agents have further advantages in use over the fatty alkyl-ammonium salts.

They give completely clear colorless solutions in water even at room temperature. The viscosity of these solutions is low even at concentrations of 50 to 80 per cent by weight of the compounds, so that they can be sprayed at high concentrations. As a result of the absence of long alkyl radicals, the compounds do not affect the handle or appearance of the fibrous materials treated therewith and do not increase the soiling tendency, in the sense of mechanical adhesion of dirt particles to the surface of the fibers. For these reasons, the compounds are particularly suitable for the antistatic treatment of textiles which suffer heavy soiling from dust, for example net curtains, carpets, furnishing fabrics and industrial fabrics, such as dust filters, conveyor belts and drive belts which in most cases are not subjected to intensive wet washing. In addition, the absence of a long alkyl radical and hence the absence of a fatty character has the advantage that the crocking fastness of dyeings produced with disperse dyes and after-treated with the compounds of the above formula is not adversely affected even in the case of deep shades.

It is very simple to use the compounds of the above formula for the antistatic treatment of fibrous materials. The treatment is suitably carried out with aqueous solutions which are applied to the material to be treated by any desired method, for example by dipping or spraying, after which the material is dried. The application of 0.03 to 2 per cent by weight of the compounds of the above formula to the fibrous material to be provided with antistatic protection has proved appropriate. The fibrous material can be provided with the antistatic finish at any desired point in the course of its processing, or after it has been finished in other respects, or even during use. It is also possible, and frequently advantageous, to combine the antistatic finishing operation with other conventional treatment of the fibrous material, by treating the fibrous material with solutions of the compounds of the above formula which also contain, for example, softeners, lubricants, brighteners, smoothing agents or wetting agents. Examples of such known agents are quaternary fatty alkyl-ammonium or fatty alkyl-sulfonium compounds, fatty acid esters, fatty acid alkylamides, tertiary or quaternary fatty acid amide-amines, fatty alkyl sulfates, sulfo-

nation products of natural fats of animal or vegetable origin, oxyalkylation products of fatty acids, sulfonate salts of alkylated aromatics, sulfuric acid ester salts of fatty alcohols and of partial fatty acid esters of polyhydric alcohols, salts of partial phosphoric acid esters, and dispersions of polyethylene and other vinyl compounds, such as copolymers of butyl acrylate, quaternary vinylimidazole and methylolacrylamide.

Apart from the treatment of fibrous materials, the compounds of the above formula have proved outstandingly successful in the antistatic surface treatment of non-fibrous articles of any materials which tend to build up an electrostatic charge, especially of materials usually referred to as plastics or resins. Here again, aqueous solutions are suitable and these can again be applied by dipping or spraying, but can also be spread by rubbing the surface to be protected with an impregnated cloth. In this way it is possible to provide, for example, films, phonograph records, lighting appliances, refrigerators, radio cabinets and plastics-veneered furniture with antistatic surface protection.

Tables 1 and 2 show the antistatic action of the compounds on textile material. The data are determined as follows:

5 25 5 g of continuous filament of polycaprolactam (dtex 67 f 12 Z) or polyethylene terephthalate (dtex 75 f 24) are wound up on a winch of 120 cm circumference. This material is treated - depending on the example - with 0 g/l, 0.5 g/l, 1 g/l or 2 g/l of antistatic agent at pH 5 to 6 for 15 minutes at 45°C, using a liquor ratio of 30:1. The material is then centrifuged until the wet pick up is 60 per cent, and is dried at 80°C. Because of the absence of any substantivity, the amount applied to the fiber corresponds to that calculated.

30 35 The hank is wrapped with a strong thread at one end and is cut open at the other end. After conditioning, the hank is repeatedly drawn through a brass die of 4.5 mm diameter until the charge has reached a maximum, and is then held in a brass half-cylinder of 80 mm diameter and 500 mm length, connected to an electrostatic voltage meter (Static-Voltmeter supplied by Rothschild, Switzerland). The potential is read off in volts.

40 40 The hanks are heat-treated in a through-circulation dryer.

TABLE 1

| Product code                        | Electrostatic charge of polycaprolactam hanks in volts at 20°C and 65% relative atmospheric humidity |                                        | Hank stored 5 minutes at 180°C       |                                      |                                |               |
|-------------------------------------|------------------------------------------------------------------------------------------------------|----------------------------------------|--------------------------------------|--------------------------------------|--------------------------------|---------------|
|                                     | Reaction product of                                                                                  |                                        | Hank before heat exposure            |                                      | Hank stored 5 minutes at 180°C |               |
|                                     | 1 mole of quaternizing agent                                                                         | 1 mole of amine                        | treated with g/l of active substance | treated with g/l of active substance | 0 (untreated)                  | 0 (untreated) |
| Examples according to the invention |                                                                                                      |                                        |                                      |                                      |                                |               |
| A                                   | Dimethyl sulfate                                                                                     | Tris-(2-hydroxyethyl)-amine            | +1,300                               | 0                                    | 0                              | +1,000        |
| B                                   | Methyl chloride                                                                                      | "                                      | "                                    | 0                                    | 0                              | "             |
| C                                   | 2-Chloroethanol                                                                                      | "                                      | "                                    | +50                                  | 0                              | "             |
| D                                   | Benzyl chloride                                                                                      | "                                      | "                                    | +100                                 | 0                              | "             |
| E                                   | p-Toluenesulfonic acid methyl ester                                                                  | "                                      | "                                    | +200                                 | 0                              | "             |
| F                                   | 0.5 mole of 1,4-dichlorobutane                                                                       | "                                      | "                                    | +50                                  | 0                              | "             |
| G                                   | Dimethyl sulfate                                                                                     | N-Methyl-bis-(2-hydroxyethyl)-amine    | "                                    | +50                                  | 0                              | "             |
| H                                   | Methyl chloride                                                                                      | "                                      | "                                    | +50                                  | 0                              | "             |
| K                                   | Dimethyl sulfate                                                                                     | N-(n-Butyl)-bis-(2-hydroxyethyl)-amine | "                                    | +200                                 | 0                              | "             |
| L                                   | Methyl chloride                                                                                      | "                                      | "                                    | +200                                 | 0                              | "             |
| Comparative                         | I                                                                                                    | Dimethyl sulfate                       | N-Dimethyl-(2-hydroxyethyl)-amine    | +1,300                               | +1,100                         | +1,000        |
|                                     |                                                                                                      |                                        |                                      |                                      | +1,000                         | +1,000        |

TABLE 1-continued

| Product code | Electrostatic charge of polycaprolactam hanks in volts at 20°C and 65% relative atmospheric humidity |                                     | Hank before heat exposure            |     | Hank stored 5 minutes at 180°C       |               |     |                |
|--------------|------------------------------------------------------------------------------------------------------|-------------------------------------|--------------------------------------|-----|--------------------------------------|---------------|-----|----------------|
|              | Reaction product of                                                                                  |                                     | treated with g/l of active substance |     | treated with g/l of active substance |               |     |                |
|              | 1 mole of quaternizing agent                                                                         | 1 mole of amine                     | 0 (untreated)                        | 0.5 | 1.0                                  | 0 (untreated) | 1.0 | 2.0            |
| son examples | II                                                                                                   | Methyl chloride                     | "                                    | "   | +1,200                               | +1,000        | "   | +1,100 + 800   |
|              | III                                                                                                  | p-Toluenesulfonic acid methyl ester | "                                    | "   | +1,300                               | +1,100        | "   | +1,000 + 1,000 |
|              | IV                                                                                                   | Dimethyl sulfate                    | N-Diethyl-(2-hydroxyethyl)-amine     | "   | +1,200                               | +1,100        | "   | + 900 + 700    |
|              | V                                                                                                    | Methyl chloride                     | "                                    | "   | +1,000                               | +1,100        | "   | +1,100 + 900   |
|              | VI                                                                                                   | Dimethyl sulfate                    | N-Di-n-butyl-(2-hydroxyethyl)-amine  | "   | +1,300                               | +1,000        | "   | +1,100 + 1,000 |
|              | VII                                                                                                  | Dimethyl sulfate                    | Tris-(2-hydroxyisopropyl)-amine      | "   | +1,300                               | +1,100        | "   | +1,000 + 1,000 |
|              | VIII                                                                                                 | Methyl chloride                     | "                                    | "   | +1,300                               | +1,300        | "   | + 900 + 1,000  |
|              | IX                                                                                                   | p-Toluenesulfonic acid methyl ester | "                                    | "   | +1,400                               | +1,100        | "   | +1,100 + 1,100 |

TABLE 2

| Product code                        | Electrostatic charge of PES hanks in volts at 20°C and 65% relative atmospheric humidity |                                     | Hank before heat exposure              |      | Hank stored 5 minutes at 200°C       |               |             |           |
|-------------------------------------|------------------------------------------------------------------------------------------|-------------------------------------|----------------------------------------|------|--------------------------------------|---------------|-------------|-----------|
|                                     | Reaction product of                                                                      |                                     | treated with g/l of active substance   |      | treated with g/l of active substance |               |             |           |
|                                     | 1 mole of quaternizing agent                                                             | 1 mole of amine                     | 0 (untreated)                          | 0.5  | 1.0                                  | 0 (untreated) | 1.0         | 2.0       |
| Examples according to the invention | A                                                                                        | Dimethyl sulfate                    | Tris-(2-hydroxyethyl)-amine            | +300 | 0                                    | 0             | -1,000      | 0 0       |
|                                     | B                                                                                        | Methyl chloride                     | "                                      | "    | 0                                    | 0             | "           | 0 0       |
|                                     | E                                                                                        | p-Toluenesulfonic acid methyl ester | "                                      | +50  | 0                                    | "             | -50         | 0 0       |
|                                     | G                                                                                        | Dimethyl sulfate                    | N-Methyl-bis-(2-hydroxyethyl)-amine    | "    | 0                                    | 0             | "           | 0 0       |
|                                     | K                                                                                        | Dimethyl sulfate                    | N-(n-Butyl)-bis-(2-hydroxyethyl)-amine | "    | +50                                  | 0             | "           | -100 0    |
|                                     | I                                                                                        | Dimethyl sulfate                    | N-Dimethyl-(2-hydroxyethyl)-amine      | +300 | +200                                 | +100          | -1,000      | -500 -600 |
|                                     | II                                                                                       | Methyl chloride                     | "                                      | "    | +200                                 | +200          | "           | -800 -200 |
|                                     | VII                                                                                      | Dimethyl sulfate                    | Tris-(2-hydroxyisopropyl)-amine        | +200 | +200                                 | "             | -700 -600   |           |
|                                     | VIII                                                                                     | Methyl chloride                     | "                                      | +300 | +300                                 | "             | -800 -300   |           |
|                                     | IX                                                                                       | p-Toluenesulfonic acid methyl ester | "                                      | +350 | +200                                 | "             | -1,000 -800 |           |

## EXAMPLE 1

A polyamide-6 knitted fabric is treated on a dyebeck using a dilute liquor (liquor ratio 30:1), with an 0.05% strength solution of N-methyl-tri-(2-hydroxyethyl)-ammonium chloride at pH 6 and approximately 40°C for 10 minutes. After centrifuging to about 30% residual moisture content, and drying, the fabric is thermoset at 180° to 200°C. A polyamide material treated in this way does not build up any electrostatic charge during subsequent processing, such as lapping and making-up, or during use.

## EXAMPLE 2

The surface of a polystyrene molding is sprayed with a 1% strength aqueous solution of N-dimethyl-bis-(2-hydroxyethyl)-methosulfate which contains 0.05% of sodium hexylheptylnaphthalenesulfonate to give better

wettability. After drying, the molding is antistatic; it shows no tendency to build up an electrostatic charge when rubbed and therefore does not attract dust from the atmosphere.

## EXAMPLE 3

A surface coated with a synthetic resin lacquer based on polyacrylic acid esters is wiped dry, with gentle pressure, with a cotton cloth which is impregnated with a 20% strength aqueous solution of N-benzyl-tri-(2-hydroxyethyl)-ammonium methosulfate. This treatment transfers a slight amount of the substance onto the synthetic resin surface so that the latter is now antistatic and does not attract dust.

We claim:

1. Fibrous material provided with an antistatic finish with 0.03 to 2 per cent by weight, based on the fibrous

material, of at least one ammonium salt of the formula



where  $\text{X}^-$  is one equivalent of an anion of a water-soluble acid, Q is hydroxalkyl of 2 or 3 carbon atoms, alkyl of 1 to 6 carbon atoms, benzyl or the radical

5



A is alkylene of 2 to 6 carbon atoms and R is hydroxalkyl of 2 or 3 carbon atoms, alkyl of 1 to 6 carbon atoms or benzyl.

2. A fibrous material as set forth in claim 1 wherein 10 said fibrous materials are prepared from polyesters, polyamides, acrylonitrile polymers, polyolefins or polyvinyl compounds.

\* \* \* \* \*

15

20

25

30

35

40

45

50

55

60

65